

Feb. 10, 1970

SUSUMU GODA ET AL

3,494,808

PROCESS FOR MANUFACTURING TOUGH STEEL

Filed Jan. 14, 1964



**INVENTORS.**

Susumu Goda  
Hisashi Gondo  
Isao Kimura  
Suehiro Hiyoshi  
Akira Yonei  
Hiroki Masumoto

*By Wendworth, Lind and Porath, atty.*

# United States Patent Office

3,494,808  
Patented Feb. 10, 1970

## 1

3,494,808

PROCESS FOR MANUFACTURING TOUGH STEEL  
Susumu Goda, Hisashi Gondo, Isao Kimura, Suehiro  
Hiyoshi, Akira Yonei, and Hiroki Masumoto, Kitakyu-  
shu, Fukuoka, Japan, assignors to Yawata Iron & Steel  
Co., Ltd., Tokyo, Japan, a Japanese corporation

Filed Jan. 14, 1964, Ser. No. 337,562

Claims priority, application Japan, Jan. 18, 1963,  
38/2,228

Int. Cl. C21d 7/14; C22c 39/30  
U.S. Cl. 148—12

4 Claims

This invention relates to a process for manufacturing tough steel, more particularly, a process for manufacturing tough steel above 15 mm. thick for use as structural steel.

Heretofore, a method is known of improving the strength of tough steel by adding niobium or vanadium thereto. However, the tough steel prepared by this known method loses rapidly the toughness to such an extent, when the thickness of the steel is increased, that it becomes difficult to obtain an impact value at 0° C. according to the V-notch Charpy impact testing method as of above 3.0 kgm./cm.<sup>2</sup>, which is generally required for use in structural steels. Therefore, it is not on record that any tough steel above 15 mm. thick has been practically used as structural steel, and the manufacture of tough steel of such thickness has been regarded as almost impossible.

As conventional tough steel is prepared by heating and rolling treatments at a temperature of above 1,250° C., bainites increase in its crystal texture, when the thickness of the steel exceeds 15 mm., whereby the toughness of the steel is lost rapidly without effecting refinement of crystal grains.

To cite an example, a steel having the thickness of 25 mm. and containing one of niobium, tantalum and vanadium, which has been treated at a temperature of above 1,250° C., shows an impact value of 1 to 1.5 kgm./cm.<sup>2</sup>. Accordingly, the steel of this kind has been deemed to be unsuitable for wide use as a tough steel.

The present invention is based on the observation that certain relationships exist between acid-soluble niobium and acid-insoluble niobium contained in steel. That is, acid-soluble niobium, which is mainly solid-dissolved in the steel, is the cause of improving the strength of the steel due to hardening caused by the solid-solution, and acid-insoluble niobium, which is deposited mainly as carbide and partly as nitride, is that which refines the crystal grains of the steel and thereby improves the toughness thereof. In analyses made by the inventors the fact has been discovered that both kinds of niobiums keep the specific equilibrium values between them, which are mainly to be determined by the heating temperature and heating time and which undergo substantially no change during the rolling process and the cooling process after the rolling, unless intentionally slow cooling is carried out. This fact is entirely unknown in any known literature.

In addition, according to the literature it was said that niobium compounds contained in the steel would be completely decomposed and solid-dissolved at a temperature of about 900° C., when they are in the composition range as specified by the present invention. However, by the present invention it was found out that acid-insoluble niobium will increase as the heating temperature will be higher and reach the maximum at a temperature of 900°

## 2

C. and then will begin to decrease immediately before 1,100° C.

Thus, the present invention is the first in obtaining the deposition of niobium compounds at such a high temperature as above mentioned and in utilizing the effects thereof. The same phenomenon may be perceived also in case of tantalum and vanadium. The present invention has succeeded in achieving both the desired strength and toughness of the steel by controlling the solid-solution and deposition of these elements, and thereby the manufacture of a tough steel above 15 mm. thick, which has been heretofore regarded as almost impossible, was made possible.

The object of the present invention is to provide a method of manufacturing a tough structural steel which possesses both properties of strength and toughness.

Another object of the present invention is to provide a method of manufacturing tough steel above 15 mm. thick which possesses both properties of strength and toughness.

Other objects of the present invention will be made clear by the following description and in reference to the attached drawing.

The single figure of drawing shows an equilibrium curve between the acid-insoluble niobium deposited in the steel and the total niobium at various heating temperatures.

The steels to be used in the present invention are those obtained by adding one or more selected from the group consisting of niobium, tantalum and vanadium in an amount of 0.02% to 0.20% in total to an ordinary carbon steel containing less than 0.40% C, Si and Mn in an amount to be contained in making steel respectively, or to a ferrite-pearlite steel similar to the above ordinary carbon steel. In case higher strength is particularly required, nitrogen should be contained in an amount less than 0.02%.

The steel containing more than 0.4% C is not suitable for the present invention, because C content of more than 0.40% will reduce the impact value. The contents of Si and Mn should be limited to those incidental to the manufacture of steel. If one or more of niobium, tantalum or vanadium is or are contained in an amount less than 0.02% in total, the effect of adding these elements cannot be displayed. If more than 0.20%, the impact value will be lowered.

According to the method of the present invention, in which the steel specified as above is heated and hot-rolled at the specified temperatures, a tough steel having sufficient low temperature strength and toughness may be obtained, even if the thickness of the steel exceeds 15 mm. Even heretofore, a tough steel itself, to which niobium, tantalum and vanadium were added, could be obtained by hot-rolling the steel to the desired dimension and shape. However, in the conventional method, the heating temperature was above 1,250° C. in general, and the rolling temperature has been also determined only in view of the easiness of plasticity.

On the other hand, the finish temperature of rolling was above 950° C. in case of rolling a relatively large-sized steel and about 900° or 850° C. even in case of rolling small-sized one.

The present invention is characterized by controlling the amount of solid-solution of acid-soluble niobium and the amount of deposition of acid-insoluble niobium.

That is to say, as shown in the aforesaid curve, acid-insoluble niobium increases gradually in accordance with the rise in the heating temperature and reaches the maximum at 900° C. and then again decreases gradually at a temperature range of immediately before 1,100° C. Therefore, it is possible to effectively control the amount of deposition by regulating the heating temperature.

As already mentioned, acid-insoluble niobium is deposited mainly in the form of carbide or partly of nitride. But, the amount of deposition is desirable to be 30% to 80% by weight, or more preferably 50% by weight of the total niobium.

As seen from the curve in the attached drawing, there are two sections in the curve which show the range of the deposition of acid-insoluble niobium in an amount of 30% to 80% of the total niobium, corresponding to the range of the heating temperature of 550° to 800° C. and that of 1,100° to 1,220° C., respectively. Correspondingly, the inventors have discovered two methods to attain the object of the present invention, that is, to obtain a tough steel possessing both properties of strength and toughness, irrespective of the thickness thereof, in which acid-insoluble niobium is deposited in an amount of 30% to 80% by weight of the total niobium. In general, the above mentioned two methods are as follows:

I. The steel slab containing less than 0.40% C by weight, less than 1.5% Mn by weight and one or more selected from the group consisting of niobium, tantalum and vanadium in an amount of 0.02% to 0.20% by weight in total is heated at a temperature of 1,100° to 1,220° C. for at least 15 minutes and immediately thereupon the thus heated slab is hot-rolled.

II. The steel slab specified as above mentioned is treated according to the conventional method, in which it is heated at a temperature above 1,250° C. and then the thus heated slab is hot-rolled, and then the hot-rolled slab is heated again at a temperature of 550° to 800° C. for at least 15 minutes.

By either of these two methods a tough steel of more than 15 mm. thick, which possesses both properties of strength and toughness, could be obtained.

The above steel slab may be prepared by the conventional method, in which a molten steel containing the elements as specified in the present invention is cast into an ingot and the ingot is made to a slab.

The time of heating the slab at a temperature of 1,100° to 1,220° C. or of 550° to 800° C., that is, at least 15 minutes, is a time necessary for effecting the deposition of acid-insoluble niobium or tantalum or vanadium in an amount of 30% to 80% by weight respectively.

The present invention will be explained more in detail by the example. Table I shows chemical compositions of specimens of steels prepared by a basic open-hearth furnace, and Table II the relationships between the compositions of steels and the impact values at 0° C. of said steels treated as follows:

The steels were heated at a temperature of 1,200° C. and immediately thereupon hot-rolled with a finish temperature of 900° C.

In the specimens D, F and G nitrogen has been added. No nitrogen has been added in the specimens which contained less than 0.006% N<sub>2</sub>.

TABLE II.—MECHANICAL PROPERTIES (WHEN THE STEEL HAS BEEN HEATED AT 1,200° C. AND ROLLED WITH A FINISH TEMPERATURE OF 900° C.) 25 MM. THICK

|    |           | Yielding point<br>(kg./mm. <sup>2</sup> ) | Tensile strength<br>(kg./mm. <sup>2</sup> ) | Elongation<br>(Percent) | Impact value at<br>0° C.<br>(kg.m./cm. <sup>2</sup> ) |
|----|-----------|-------------------------------------------|---------------------------------------------|-------------------------|-------------------------------------------------------|
| 10 | Specimen: |                                           |                                             |                         |                                                       |
|    | A         | 35                                        | 49                                          | 32                      | 15                                                    |
|    | B         | 39                                        | 55                                          | 28                      | 6                                                     |
|    | C         | 41                                        | 54                                          | 27                      | 9                                                     |
|    | D         | 43                                        | 59                                          | 24                      | 5                                                     |
|    | E         | 42                                        | 55                                          | 27                      | 8                                                     |
|    | F         | 48                                        | 65                                          | 21                      | 4                                                     |
|    | G         | 40                                        | 59                                          | 24                      | 4                                                     |
|    | H         | 44                                        | 62                                          | 20                      | 4                                                     |
|    | I         | 49                                        | 65                                          | 17                      | 1                                                     |
|    | J         | 50                                        | 68                                          | 18                      | 4                                                     |
|    | K         | 51                                        | 70                                          | 15                      | 2                                                     |
|    | L         | 43                                        | 56                                          | 26                      | 7                                                     |

As seen from the above table manganese improves the impact value without impairing the strength. However, if the content of manganese is more than 1.5%, the steel becomes brittle and the weldability will be impaired.

Therefore, it should be limited to below 1.5% by weight. Nitrogen improves strength of the steel, but will reduce the impact value when it increases, and makes the steel brittle when the content thereof exceeds 0.02%. Therefore, if the steel possesses already the desired strength, it is not necessary to especially add nitrogen. Carbon will reduce the impact value, if the content thereof is more than 0.40%.

On the other hand, even if the other elements are contained in the specified ranges as above mentioned, the addition of niobium, tantalum or vanadium of more than 0.20% by weight in total will reduce largely the impact values, while no effect of adding these elements will be displayed, if the addition of any of them is less than 0.02% by weight in total.

Table III shows the relationships between the heating and rolling conditions of specimen No. E and mechanical properties thereof.

TABLE III.—RELATIONSHIPS BETWEEN THE HEATING AND ROLLING CONDITIONS AND MECHANICAL PROPERTIES (EXAMPLE OF E) 25 MM. THICK

| Finish temperature of rolling, °C. | Heating temperature, °C. |         |         |        |        |
|------------------------------------|--------------------------|---------|---------|--------|--------|
|                                    | 1,100                    | 1,150   | 1,200   | 1,220  | 1,250  |
| 1,050                              | 50 (2)                   | 52 (2)  | 53 (2)  | 54 (2) | 55 (1) |
| 1,000                              | 51 (8)                   | 52 (6)  | 54 (4)  | 55 (4) | 59 (1) |
| 950                                | 52 (15)                  | 53 (10) | 55 (8)  | 56 (4) | 60 (1) |
| 900                                | 52 (14)                  | 53 (10) | 55 (8)  | 56 (3) | 61 (1) |
| 850                                | 53 (15)                  | 54 (11) | 56 (10) | 57 (4) | 60 (1) |
| 800                                | 54 (15)                  | 55 (13) | 57 (9)  | 56 (4) | 61 (2) |

Numbers in parentheses designate the impact value at 0° C. (kg. m./cm.<sup>2</sup>).

Numbers outside parentheses show the tensile strength (kg./mm.<sup>2</sup>).

As seen from Table III, if the heating temperature exceeds 1,220° C., the tensile strength will be elevated, but

TABLE I.—CHEMICAL COMPOSITIONS (PERCENT BY WEIGHT)

| Specimen: | Carbon | Silicon | Manganese | Niobium | Tantalum | Vanadium | Nitrogen |
|-----------|--------|---------|-----------|---------|----------|----------|----------|
| A         | 0.09   | 0.07    | 1.07      | 0.04    | 0.02     | .....    | 0.004    |
| B         | 0.18   | 0.06    | 0.82      | 0.05    | .....    | .....    | 0.004    |
| C         | 0.18   | 0.09    | 1.13      | .....   | .....    | 0.06     | 0.005    |
| D         | 0.19   | 0.10    | 1.22      | 0.07    | .....    | .....    | 0.015    |
| E         | 0.18   | 0.05    | 1.25      | 0.06    | .....    | .....    | 0.008    |
| F         | 0.19   | 0.08    | 1.28      | .....   | .....    | 0.07     | 0.016    |
| G         | 0.19   | 0.08    | 1.22      | 0.07    | .....    | 0.05     | 0.016    |
| H         | 0.35   | 0.08    | 0.91      | 0.04    | .....    | .....    | 0.006    |
| I         | 0.42   | 0.08    | 0.97      | 0.04    | .....    | .....    | 0.005    |
| J         | 0.17   | 0.07    | 1.35      | .....   | .....    | 0.18     | 0.004    |
| K         | 0.15   | 0.06    | 1.28      | .....   | .....    | 0.23     | 0.004    |
| L         | 0.16   | 0.07    | 1.24      | .....   | 0.07     | .....    | 0.004    |

the impact value will be reduced. If the finish temperature of rolling exceeds 1,000° C., the ferrite grains and pearlite spacing cannot be refined, thereby both impact value and strength will be reduced. Therefore, the heating temperature should be in a range of 1,100° to 1,220° C. and the finish temperature of rolling should be below 1,000° C.

TABLE IV.—RELATIONSHIPS BETWEEN REHEATING AFTER ROLLING AND MECHANICAL PROPERTIES (EXAMPLE OF E) 25 MM. THICK

Reheating temperature before rolling, 1,250° C.  
Final temperature of rolling, 900° C.

| Reheating temperature (° C.): | Tensile strength (kg./mm. <sup>2</sup> ) | Impact value (kg. m./cm. <sup>2</sup> ) |
|-------------------------------|------------------------------------------|-----------------------------------------|
| As welded.....                | 61                                       | 1                                       |
| 400.....                      | 59                                       | 1                                       |
| 500.....                      | 58                                       | 2                                       |
| 600.....                      | 57                                       | 4                                       |
| 700.....                      | 54                                       | 10                                      |
| 800.....                      | 53                                       | 14                                      |
| 900.....                      | 51                                       | 15                                      |

As seen from Table IV, in the slab, which has been subjected to a heating treatment at a temperature of 1,250° C. as according to the conventional method, the ratio of amount of deposition to amount of solid-solution of niobium, tantalum or vanadium necessary for obtaining both strength and toughness as aimed at by the present invention could not be obtained. Consequently, the impact value thereof was very low.

Therefore, in order to obtain 30% to 80% of the deposition of acid-insoluble niobium, tantalum or vanadium, it was necessary to reheat the slab heated and hot-rolled according to the conventional method at a temperature of 550° to 800° C. as specified by the present invention.

By thus reheating the slab both strength and toughness as desired could be obtained. But if the reheating temperature is not in the above mentioned range, the object of the present invention cannot be attained.

What we claim is:

1. A method for producing tough steel having a thick-

ness exceeding 15 mm. comprising heating steel consisting of less than 0.4% by weight C, less than 1.5% by weight Mn and from 0.02 to 0.20% by weight Ta, the rest being essentially iron, at a temperature of 1,100 to 1,220° C., for at least 15 minutes, and thereupon subjecting the heated steel to hot-rolling with a finishing temperature of less than 1,000° C.

2. A method for producing tough steel having a thickness exceeding 15 mm. comprising making molten steel consisting of less than 0.40% by weight C, less than 1.5% by weight Mn and 0.02 to 0.20% by weight Ta, the rest being essentially iron, casting the molten steel into form, making a slab from the ingot, then heating said slab at a temperature of 1,100 to 1,220° C. for at least 15 minutes, and thereupon subjecting the heated slab to hot rolling with a finishing temperature of below 1,000° C.

3. A method for producing tough steel having a thickness exceeding 15 mm. comprising heating steel consisting of less than 0.4% by weight C, less than 1.5% by weight Mn and from 0.02 to 0.20% by weight V, the rest being essentially iron, at a temperature of 1,100 to 1,220° C., for at least 15 minutes, and thereupon subjecting the heated steel to hot-rolling with a finishing temperature of less than 1,000° C.

4. A method for producing tough steel having a thickness exceeding 15 mm. comprising making molten steel consisting of less than 0.40% by weight C, less than 1.5% by weight Mn and 0.02 to 0.20% by weight V, the rest being essentially iron, casting the molten steel into form, making a slab from the ingot, then heating said slab at a temperature of 1,100 to 1,220° C. for at least 15 minutes and thereupon subjecting the heated slab to hot rolling with a finishing temperature of below 1,000° C.

#### References Cited

The Making, Shaping and Treating of Steel, seventh edition, 1957, pp. 386-387.

L. DEWAYNE RUTLEDGE, Primary Examiner

W. W. STALLARD, Assistant Examiner